# EUROPEAN PATENT SPECIFICATION

(11) **EP 2 990 527 B1**
(45) Date of publication and mention of the grant of the patent: **07.02.2018**
(21) Application number: 15468007.8
(22) Date of filing: 11.08.2015
(51) Int. Cl.: D06M 11/79, D06M 23/08, D06M 101/06

(54) **A PROCESS FOR PREPARING OF COTTON TEXTILES HAVING SELF-CLEANING AND WASHING RESISTANT PROPERTIES**
VERFAHREN ZUR HERSTELLUNG VON BAUMWOLLTEXTILIEN MIT SELBSTREINIGUNGS- UND WASCHBESTÄNDIGKEITSEIGENSCHAFTEN
PROCÉDÉ DE PRÉPARATION DE TEXTILES EN COTON AYANT DES PROPRIÉTÉS DE RÉSISTANCE AU LAVAGE ET AUTONETTOYANTES

(30) Priority: 18.08.2014 SI 201400289
(43) Date of publication of application: 02.03.2016
(73) Proprietor: Kemijski Institut, 1000 Ljubljana (SI); Univerza v Ljubljani, 1000 Ljubljana (SI)
(72) Inventor: Zorko, Milena, 8312 Podbocje (SI); Simoncic, Barbara, 3311 Sempeter (SI); Vasiljevic, Jelena, 1000 Ljubljana (SI); Tomsic, Brigita, 6230 Postojna (SI); Jerman, Ivan, 3305 Vransko (SI); Gaberscek, Miran, 1230 Domzale (SI)
(74) Representative: Macek, Gregor

(56) References cited:
- LENG BOXUN ET AL: "Superoleophobic Cotton Textiles", LANGMUIR, AMERICAN CHEMICAL SOCIETY, NEW YORK, NY; US, vol. 25, no. 4, 22 January 2009 (2009-01-22), pages 2456-2460, XP002601745, ISSN: 0743-7463, DOI: 10.1021/LA8031144
- H. F. HOEFNAGELS ET AL: "Biomimetic Superhydrophobic and Highly Oleophobic Cotton Textiles", LANGMUIR, vol. 23, no. 26, 27 September 2007 (2007-09-27), pages 13158-13163, XP55243993, NEW YORK, NY; US ISSN: 0743-7463, DOI: 10.1021/la702174x
- JUN LIANG ET AL: "Transformation of hydrophilic cotton fabrics into superhydrofobic surfaces for oil/water separation", THE JOURNAL OF THE TEXTILE INSTITUTE, TAYLOR & FRANCIS, vol. 104, no. 3, 10 August 2012 (2012-08-10), pages 305-311, XP001581545, ISSN: 0040-5000, DOI: HTTP://DX.DOI.ORG/10.1080/00405000.2012.72 1207
- BAE G Y ET AL: "Superhydrophobicity of cotton fabrics treated with silica nanoparticles and water-repellent agent", JOURNAL OF COLLOID AND INTERFACE SCIENCE, ACADEMIC PRESS, NEW YORK, NY, US, vol. 337, no. 1, 22 April 2009 (2009-04-22), pages 170-175, XP027597754, ISSN: 0021-9797, DOI: 10.1016/J.JCIS.2009.04.066 [retrieved on 2009-05-03]

## Description

### Field of invention

The invention relates to a process for the preparation of self-cleaning wash-resistant and air-permeable superhydrophobic and oleophobic cotton textiles. The coating is applied *in-situ* to the surface of the cotton textile. This resulted in water sliding angles smaller than 15 degrees even after ten washings.

### Background of the invention

Cotton fibres are natural cellulosic fibres that are widely used as a raw material for the manufacturing of various textile products. Their attractiveness is directly related to the chemical structure and morphological characteristics of the cellulosic fibres. These fibres are pleasant to the touch and exhibit a hydrophilic character to ensure product comfort, respiratory activity, and aesthetic appearance. The fibres are biodegradable, which, in terms of ecology and sustainable development, is their major advantage over synthetic fibres.

Cotton fibres have been gaining attention as components in the production of specialized high-tech textiles; this is due to their advantages and successfully outcompeting ecologically less acceptable synthetic fibres. Such high-tech materials include bio-mimetic self-cleaning textiles, which must ensure simultaneous wetting resistances for a variety of polar and nonpolar liquids, in addition to air and water vapour permeabilities. These requirements can only be achieved by careful chemical modifications of the cellulosic fibre surface.

The use of textiles that are easy on the skin and, at the same time, offer the user welfare and protection against the environment are very common in everyday life. Such fabrics are on the one hand suitable for sports and leisure (e.g., obstacle courses, mountaineering, cross-country running, downhill skiing, motocrossing, mountain biking) and, on the other hand, serve as protective technical textiles. Technical textiles are used by professionals who frequently encounter water and soilage (e.g., butchers, plumbers, hairdressers, bricklayers, fine mechanics or firefighters). All of the mentioned users are also likely to be physically active, which results in sweating and may also stain the textiles. In such cases, it is recommended that the textile allows for the passage of body sweat, so that end users are not completely drenched with sweat for long periods.

Superhydrophobicity and oleophobicity are basic properties of a solid surface that are dependent on the chemical composition and the surface roughness of a substrate. Chemical composition determines surface free energy and, consequently, surface wettability. Micro- and nanostructured surfaces can further influence wettability, if the roughness is inappropriate.

EP 2,589,578 A1 patent application shows that a reduction in surface wettability can be achieved by the derivatives of catechols. In addition to a low surface free energy, the fluorinated catechol derivatives have been known to form vesicles (70 nm) or capsules with a hollow core 200 to 1000 nm in size, which increase microstructure. This combination of features enables the preparation of surfaces, such as carbon nanotubes, iron oxide nanoparticles and mesoporous silica, with water-repellent properties.

In US Patent Application 20020192385A1 Jenkner et al. describe a method for the application of hydro- and oleophobic fluorinated coatings on polymeric substrates pre-treated by physical methods (plasma, corona discharge, and electromagnetic radiation). In the next step, fluorinated silanes are applied to the activated surface with bonding promoters (metal oxides).

U.S. Patent 7,732,497 B2 discloses the use of pre-prepared surface-treated particles for the preparation of a liquid repellent layer. A minimum of two particle sizes are used, and at least one particle surface is further functionalized by alkyl chains.

US 7,985,475 B2 patent describes the preparation of superhydrophobic coatings by placing well-defined silicon nano-fibres on a surface coated with exogenous hydrophobic or amphiphilic materials. In the patent, fluorinated molecules are also used to achieve hydrophobic properties.

U.S. Patent 8,541,056 B2 discloses the preparation of water-repellent textiles by mechanical abrasion. The previously abraded substrates are coated with colloidal dispersions of various metal oxides (commercial products) and cross-linked using isocyanate compounds, which usually form at the end of polyurethane bonds.

The preparation of water-repellent textiles is also possible by integrating fumed SiO₂ particles with the fibres through the use of binders without formaldehyde, as indicated in US patent application 20110287245. Alkali metal salts of phosphorous are used as a catalyst for polymerization, which allows the matrix and the cellulose fibres to bond together. A method for preparing water-repellent coatings also includes the use of SiO₂ particles prepared from dimethyldichlorosilanes and coated with polycarboxylic acids.

US patent application 20110250422A1 discloses the use of a porous matrix built from fluorosilanes for the preparation of hydro- and oleophobic coatings. The main significance of the coating, given the pore size and the distribution of pores by volume, is its suitable surface roughness in combination with a low surface free energy that are provided by the building blocks of the porous structures. The coatings can also be used to reduce adhesion, which provides the surfaces with a self-cleaning effect.

Bae et al. (Colloid Interface Sci., 337 (2009) 170-175) prepare a water-repellent layer on textiles, mainly because of their good qualities, such as tenderness, comfort, biodegradability, and low cost, as well as the possibility of applying the layer to casual wear. To produce the aforementioned textile coatings, the authors combine SiO₂ particles with a chemical-based low-cost water repellent. By using this method, they obtain a static contact angle for water of 140°. Oil repellent properties, which are acquired by measuring the static contact angles for a series of n-alkanes (C6-C25), are not specified.

The preparation of cotton textiles with high static contact angles for water (up to 150°) and n-hexadecane (near 120°) is possible with surface finishes prepared from alkoxy-functionalized PDMS in combination with perfluorinated alkoxy silanes. This low surface free energy of these coatings prevents the adhesion of bacteria to the surface, thereby imparting passive antimicrobial properties to cotton textiles (Vilćnik A. et al Langmuir, 25 (2009) 5869-5880).

Ma et al. (J. Colloid Interface Sci., 392 (2013) 194-200) report on the use of a single-stage emulsion to prepare monodisperse polysiloxane spherical particles surface-functionalized with a variety of organic groups. In addition to water-repellency, the authors analyse the influence of the organic groups on the properties of the coatings, e.g., thermal stability. The purpose of generating particles on the surface of cotton was to imitate the surface structure of a lotus leaf.

Stöber et al. (J. Colloid Interface Sci., 26 (1968) 62-69) previously reported on the mechanism of amorphous SiO₂ particle formation and proposed a series of chemical reactions that resulted in the controlled growth of uniformly sized spherical particles.

Leng et al describe in "Superoleophobic Cotton Textiles" (Langmuir 2009, 25, 2456-2460) the process for preparation of superoleofobic cotton textiles. The process includes the following steps: applying in situ generated silica particles which are covalently bonded on the cotton fibers. In the next step the adsorption of silica nanoparticles occurs, wherein the adsorption process is driven by electrostatic attraction (by treating with 3-aminopropyl-triethoxysiloxane and hydrochloric acid the surface charge is turned positive due to the protonation of amine groups) and the fabric is dipped into dispersion of negatively charged silica nanoparticles. The obtained roughened structure is stabilized by SiCl₄ and in the next step the surface is modified with perfluoroalkyl silane.

H. F. Hoefnagels et al describe in "Biomimetic superhydrophobic and highly oleophobic cotton textiles" (Langmuir 2007, 23, 13158-13163) biomimetic process for the preparation of superhydrophobic cotton textiles. By in-situ introducing silica particles to cotton fibres to generate a dual-size surface roughness, followed by hydrophobization with polydimethylsiloxane, normally hydrophilic cotton has been tutrned superhydrophobic.

Liang et al describe in "Transformation of hydrophilic cotton fabrics into superhydrophobic surfaces for oil/water separation (The Journal of The Textile Institute 2012, 104, 305-311) the preparation process wherein silica hydrosols are firstly prepared by water-base sol-gel method with surfactant emulsification, using tetraethoxysilane and ammonium hydroxide. Then silica hydrosols were applied to the cotton fabrics followed by the modification with silane and heat treatment.

Though modified cotton fabrics provide high contact angles for water and oil, it is necessary to wash technical cotton textiles for hygienic reasons. However, we do not want to lose the superhydrophobic, oleophobic, and self-cleaning properties that prevent the retention of various emulsions on the surface of cotton fabrics during the washing process. According to the literature, there are no reports on washing resistant cotton textiles prepared by SiO₂ spherical particles, nor is there mention of the *in-situ* modification of cotton by SiO₂ particles for the production of the aforementioned textiles.

The present invention relates to a process that enables the preparation of wash-resistant, air-permeable superhydrophobic, oleophobic, and self-cleaning coatings from a variety of organic-modified silanes. In the first stage of the process, pre-prepared first type of spherical SiO₂ particles are deposited, in the second stage, *in-situ* monodisperse particles of SiO₂ are formed with the use of silanes. In the next stage, the formed particles are chemically bonded to the surface of cotton textiles, which acquire a low surface energy. An appropriate surface roughness, resulting from the chemical bonding between the SiO₂ spherical particles and the cotton fibre surface, is maintained on the cotton even after four washing cycles according to ISO 105-C06: 1994 (E), which is equivalent to twenty washings in a household washing machine. The SiO₂-cotton chemical links are further consolidated by the porous structure of hardened perfluoro-modified silanes. The process enables the preparation of finishes for cotton-based textiles and products that require durable superhydrophobic and oleophobic properties in combination with a highly breathable textile, which provides air and water vapour (perspiration) permeation.

### Summary of the invention

According to the invention, the preparation of wash-resistant textiles is conducted using a wet process without compounds that release toxic formaldehyde. The process allows the chemical bonding of spherical SiO₂ particles to the cotton fibre surface, providing an appropriate surface roughness to the fabrics and is responsible for the following characteristics:
- superhydrophobicity, as determined by obtaining static contact angles for water (a 5 µL water droplet) between 160 and 170° for the finished surface of textiles and remaining as such after several consecutive washings;
- superoleophobicity, by measuring static contact angles for n-hexadecane (a droplet of n-hexadecane with a volume of 1 µL) on the textile and showing contact angles between 130 and 150°, which are maintained even after repeated washings;
- self-cleaning property, by measuring a tilt angle, which is the inclination needed for a water droplet to remove dirt from the textile surface, between 2 and 10° to a horizontal surface and exhibiting angles of less than 15° after ten household washings cycles;
- air permeability, as determined by the standard BS EN ISO 9237: 1999 after four washing cycles, which are conducted according to the standard ISO 105-C06: 1994 (E) and is the equivalent of twenty washings in a household washing machine;
- washing fastness, as exhibited by the rough surface of textiles, which are retained after washing (ISO 105-C06: 1994 (E));
- and thermal stability, as evidenced by the absence of degradation even after prolonged exposure to an elevated temperature (120 °C/30 min).

The described wash-resistant properties can be achieved only with the use of the proposed process. In the first step, we apply pre-prepared siloxane particles, which are spherical SiO₂ particles, i.e. first type of spherical SiO₂ particles. In the second step, the spherical SiO₂ particles, i.e. second type of spherical SiO₂ particles, grow *in-situ* over the cotton fibre surface covered with the spherical SiO₂ particles of the first step and form a network, thus, enabling the formation of chemical bonds between amorphous SiO₂ particles of the first step and the cotton fibre surface. These chemical bonds further consolidate in the third step and form a network with a water- and oil-repellent layer derived from a water-based precursor.

### Detailed description

According to the present invention, it is possible to produce wash-resistant, respiratory active textiles with superhydrophobic, highly oleophobic and self-cleaning properties. These textiles have a passive antibacterial protection and can be used for clothing, as in the above-described case. Superhydrophobic and oleophobic properties are derived from the roughness of a suitable double nano- and microstructured textile surface. Double roughness is achieved by applying pre-manufactured spherical SiO₂ particles to the surface of the textile, in the first step, and is supplemented by the *in-situ* formation of spherical SiO₂ particles on the surface of the textile, in the second step. According to the proposed process, the pre-manufactured spherical SiO₂ particles are responsible for the increase in the surface roughness, whereas the application of *in-situ* SiO₂ particles in the second step is unavoidable because of the lack of a chemical connection between the spherical SiO₂ particles and the cotton fibre surface. Non-bonded spherical SiO₂ particles are removed from the surface of the textile with the first washing. This disadvantage, which is inherent to the classical single step process, is eliminated by a second step. This step consists of covering and soaking the entire surface, i.e., the spherical SiO₂ particles of the first step and the fibres, with a solution of tetraethoxysilane (TEOS), base, water and alcohol, during which the *in-situ* formation of spherical SiO₂ particles of the second step with a size between 50 and 200 nm occurs. At the same time, the formation of spherical SiO₂ particles of the second step which is in a form of a thin porous coating allows the chemical bonding of spherical SiO₂ particles, deposited in the first step, to the surface of cotton. The spherical SiO₂ particles of the first step are used directly from the solution in which they have been prepared to avoid the problem of particle agglomeration, which is probable when dried particles are re-dispersed. Water- and alcohol-based dispersions in the proposed invention are characterized by a high content of cross-linked polysilsesquioxanes. Nanometre-sized siloxane spheres are responsible for the formation of a thin film of comparable thickness.

The invention is presented in detail by the figures below:
Figure 1: Scanning electron microscopy (SEM) images of cotton fibres without modification.
Figure 2: SEM images of cotton fibres modified with 200 nm SiO₂ particles.
Figure 3: SEM images of cotton fibres, modified by the operative procedure CO/AP600+IS150-FAS, after one washing cycle according to the standard ISO 105-C06: 1994 (E), which is equivalent to five washings in the household washing machine.
Figure 4: SEM images of cotton fibres, modified by the operative procedure CO/AP60+IS 150-FAS, after two washing cycles according to the standard ISO 105=C06: 1994 (E), which is equivalent to ten washings in a household washing machine.
Figure 5: SEM images of cotton fibres, modified by the operative procedure CO/AP60+IS 150-FAS, after three washing cycles in accordance with ISO 105-C06: 1994 (E), which is equivalent to fifteen washings in a household washing machine.
Figure 6: SEM images of cotton fibres, modified by the operative procedure CO/AP60+IS 150-FAS, after four washing cycles according to the standard ISO 105=C06: 1994 (E), which is equivalent to twenty washings in a household washing machine.
Figure 7: The static contact angles, *θ*, for water on cotton textiles functionalized by different implementation procedures (sample) and after a number of washings (W) According to ISO 105-C06: 1994 (E).
Figure 8: The static contact angles, *θ*, for n-hexadecane on cotton textiles functionalized by different implementation procedures (sample) and after a number of washings (W) according to ISO 105-C06: 1994 (E),
Figure 9: The tilt angles for water, a on cotton textiles functionalized by different implementation procedures (sample) and after different washings.

A process for the preparation of the wash-resistant, vapour permeable, self-cleaning, and highly hydrophobic and oleophobic cotton textiles according to claim 1, involves the following steps:
- modifying the cotton fabrics in advance with a deposition of pre-prepared first type of spherical SiO₂ particles, wherein the modification is carried out using aqueous/alcoholic dispersions of spherical SiO₂ particles 200-1000 nm in size;
- applying a second type of spherical SiO₂ particles by an *in-situ* sol-gel method, wherein the second type of spherical SiO₂ particles is grown *in-situ* on the surface of textile fibers from a colloidal nucleus disperison during which the *in-situ* formation of spherical SiO₂ particles of the second step with a size between 50-200 nm occurs, and wherein the whole surface of the textile is covered with the same bi-hierarchical roughness through the formation of a thin porous coating, which enables the chemical bonding of the first type of spherical SiO₂ particles, deposited in the first step, to the surface of cotton fabrics;
- the rough cotton surface is further consolidated by application of a sol-gel coating prepared from hydrophobic and oleophobic silanes.

### Modifying the cotton fabrics with the pre-prepared spherical SiO₂ particles

The aqueous/alcoholic dispersions of SiO₂ particles, i.e., colloidal dispersions based on tetraethoxysilane, include pre-prepared monodisperse spherical SiO₂ particles. It is desirable that at least 95% of the particles in the dispersion are the same size. The SiO₂ particle size is 200 - 1000 nm. The weight ratio of alcohol:TEOS:NH3:water is 46:2:1:5. Preparation of the particles is not the subject of the patent. According to the invention, the dispersion of SiO₂ particles is 10% by weight and is used in the first step of the process for the cotton modification, i.e., for the application of the first coating on the cotton fibre surface. The ratio of the weight of the aqueous alcoholic dispersion of SiO₂ particles and the weight of the textiles should be 1:15. After application of the dispersion of SiO₂ particles, a padder is used to squeeze the excess dispersion from the textiles while passing the textile sample between two rollers at a pressure of 0.4 bar; the fabric is then air dried at room temperature for 10 min. The advantage of the first layer is that the deposited SiO₂ particles are well separated from each other, which enables a high surface roughness of the textile. The exact parameters are very important to avoid loss of the SiO₂ particles from the surface. SiO₂ particles are preferably prepared from tetraethoxysilane, so their surface is full of free-OH bonds, which will enable chemical linking between the SiO₂ particles and the cotton fibres of the textile in the next stage.

### In-situ growth of spherical SiO₂ particles on the surface of modified SiO₂ particles and fibres

It is known that the *in-situ* growth of particles by a sol-gel method allows greater coating density after a suitable thermal treatment. In the second step, the cotton fibre surface, modified by spherical SiO₂ particles, is coated by a second layer of siloxane particles. These are spherical SiO₂ particles 50 - 200 nm in size, which are made *in-situ* by the sol-gel growth method from a colloidal nucleus dispersion. The weight ratio of alcohol:TEOS:NH₃:water is in this case 30:5:2:5. This coating enables the chemical bonding of SiO₂ particles, which were deposited on the cotton fibre surface in the first step. The reactivity of the substrate, which consists of cellulosic OH groups and surface OH groups on the spherical SiO₂ particles from the first layer, facilitates the connection to particles from the second step of the process. Simultaneously, the colloidal dispersion at the concentration described for the *in-situ* process generates uniform spherical SiO₂ particles that are sized 50 - 200 nm. The *in-situ* deposited SiO₂ spherical particles give the cotton fibre surface a double roughness, or a bi-hierarchical roughness, and at the same time secures the SiO₂ particles deposited in the first step. For the second step of the process, it is important to apply two to three times more particles, compared with the amount applied in the first step. Therefore, the smaller SiO₂ particles that are produced during the *in-situ* growth completely cover the textile surface. The weight ratio between the pre-manufactured siloxane particles used in the first step and the *in-situ* siloxane particles prepared in the second step is between 1:2 and 1:3.

### Consolidation of the rough surface of the textile by silanes

In the third step, the biomimetic surface of the textile, which has already hardened, is coated again with a thin layer of hydrophobic and oleophobic silanes, preferably from hydrolysed fluorosilane (FAS), bis [(ureapropyl) triethoxysilane] bis(propyl)-terminiran-polydimethylsiloxane (PDMSU) or a mixture of FAS and PDMSU. A 10% aqueous/alcohol solution of silane is used for the coating. This layer allows further consolidation of the biomimetic surface from the first two steps and grants the textile surface superhydrophobic, high oleophobic and self-cleaning properties. The thickness of such a thin layer may not exceed 150 nm. Hardening of the surface is possible due to the covalent bonding between the free-OH groups present on the surface of the porous coating applied in the second step and the OH groups of the hydrolysed silane. Thermal curing of the coating results in an increased density and stability, as well as an increased washing fastness.
Hydrophobic and oleophobic silanes, which are used for the hardening of the rough surfaces, are selected from the groups of perfluoroalkyl-trialkoxysilanes, perfluoroalkyl-alkyldialkoxysilanes, perfluoroalkyl-dialkylalkoxysilanes, perfluoroalkyl-trihalosilanes, perfluoroalkyl-alkyldihalosilanes, perfluoroalkyl-dialkylhalosilanes and (trialkoxysilyl)alkyl terminated polydimethylsiloxane.

The formation of individual layers with a specific particle size depends on the properties of the applied colloidal dispersions but is preferably within the conditions set out below. Various alcohols, such as methanol, ethanol, isopropanol, and butanol, should be used in the preparation of colloidal dispersions. These solvents affect the growth and size of the particles. According to the invention, additional organic-modified silanes may also be used for the preparation of SiO₂ particles in the first and second steps, such as methyltriethoxysilane, vinyltriethoxysilane, and aminopropyltriethoxysilane. Monodisperse SiO₂ particles provide a uniform roughness over the entire surface of the textile. Application can be performed by the exhaustion method, dipping, or sputter deposition.

Cotton fibres already possess their own roughness (Figure 1), but because of their chemical composition (cellulose), they are extremely hydrophilic. The surface roughness is improved by the proposed process, as shown in Figure 2. High washing fastness is provided by the *in-situ* growth of particles in the second layer and by further consolidation of the fluorosilane coating. The final coating maintains its properties after the first washing cycle, according to the standard ISO 105-C06: 1994 (E), and is equivalent to five washings in a household washing machine (Figure 3). It is slightly changed after four washing cycles (Figures 4 to 6).

The modified textile displays high hydrophobic and oleophobic properties after twenty washings with static contact angles for n-hexadecane higher than 130°. The results that indicate the preservation of the superhydrophobicity and oleophobicity are disclosed in Figures 7 and 8. These figures show the static contact angles for water and n-hexadecane as a function of the number of washing cycles, according to the standard ISO 105-C06: 1994 (E), (1W = 5x washing in a household washing machine) for the various embodiments of the invention. The extremely low sliding angles for the modified textile (Figure 9) allow rolling of the droplets and the simultaneous removal of dirt from the surface, demonstrating the self-cleaning properties.

### Examples:

The reaction conditions for the preparation of SiO₂ particles from tetraethoxysilane (TEOS 98%, Aldrich) in alcohol are as follows:
- reaction temperature, T = 60 °C;
- concentration (TEOS) = 0.2 - 1.1 mol/L;
- concentration (NH₃) = 0.3 - 1.1 mol/L;
- concentration (H₂O = 6 - 10 mol/L;
- reaction time = 1 - 3 h.

### CO/AP200-FAS

A bottle (250 mL) was filled with 130 g of ethanol and 8 g of TEOS. The solution was well mixed and allowed to stand for an additional 10 min at room temperature (RT). In the second step, a mixture of ammonia (4 g (25%)) and water (20 g) was added to the prepared solution of EtOH and TEOS. The solution was re-mixed and left for 3 h at RT. The prepared solution was used for finishing the cotton fabric. After soaking the textile in the above described reaction mixture, the fabric was squeezed with an 85% spin effect and air dried. In final step, the application of a 10% FAS solution was followed by the impregnating procedure with full soaking, squeezing with an 85% spin effect, drying at 100 °C and curing at 150 °C for 5 min.

### CO/AP200+IS150-FAS

In a bottle, a solution of 130 g ethanol and 8 g of TEOS was well mixed and allowed to stand for an additional 10 min at room temperature. Ammonia (4 g) in water (20 g) was then added to the prepared solution, which was re-mixed and left for 3 h at RT. Cotton fabric was treated in the next step by the above-described dispersion. The soaked fabric was squeezed with an 85% spin effect and air dried. The as-prepared cotton fabrics were added to a mixture of 2-propanol (100 g) and TEOS (20 g), mixed well, and left for 10 min at 50 °C. Then, a solution of ammonia (4 g) in water (20 g) was added to the TEOS solution, which was re-mixed again and left for 1 h at 50 °C. The immersed cotton textile was taken out of the reaction mixture, rinsed with water three times and dried at room temperature. This was followed by applying a 10% FAS solution, performing the impregnating procedure with full soaking, squeezing with an 85% spin effect, drying at 100 °C and curing at 150 °C for 5 min.

### CO/AP60+IS150-FAS

The solution of 130 g ethanol and 15 g of TEOS was mixed well in the bottle and allowed to stand for 10 min at 40 °C. Then, ammonia (4 g) in water (20 g) was added to the prepared solution, which was re-mixed and left for additional 1 h at 40 °C. Cotton fabric was treated in the next step by the above described dispersion. The soaked fabric was squeezed with an 85% spin effect and air dried. The as-prepared cotton fabrics were added, in the next step, to the mixture of 2-propanol (100 g) and TEOS (20 g), mixed well, and left for 10 min at 50 °C. Then, a solution of ammonia (4 g) in water (20 g) was added to the TEOS solution, which was re-mixed again and left for 1 h at 50 °C. The immersed cotton textile was taken out from the reaction mixture, rinsed with water three times and dried at room temperature. This was followed by applying a 10% FAS solution, performing the impregnating procedure with full soaking, squeezing with an 85% spin effect, drying at 100 °C and curing at 150 °C for 5 min.

### CO/AP600+IS150-FAS

The solution of 120 g ethanol and 20 g of TEOS was mixed well in the bottle and allowed to stand for 10 min at 50 °C. Then, ammonia (7 g) in water (20 g) was added to the prepared solution, which was re-mixed and left for an additional 1 h at 50 °C. Cotton fabric was treated in the next step by the above described dispersion. The soaked fabric was squeezed with an 85% spin effect and air dried. The as-prepared cotton fabric was added, in the next step, to the mixture of 2-propanol (100 g) and TEOS (20 g), mixed well, and left for 10 min at 50 °C. Then, a solution of ammonia (7 g) in water (20 g) was added to the TEOS solution, which was re-mixed again and left for 1 h at 50 °C. The immersed cotton textile was taken out from the reaction mixture, rinsed with water three times and dried at room temperature. This was followed by applying a 10% FAS solution, performing the impregnating procedure with full soaking, squeezing with an 85% spin effect, drying at 100 °C and curing at 150 °C for 5 min.

### CO/AP600+IS150-PDMSU-FAS

In a bottle, a solution of 120 g ethanol and 20 g of TEOS was mixed well and allowed to stand for 10 min at 50 °C. Then, ammonia (7 g) in water (20 g) was added to the prepared solution, which was re-mixed and left for an additional 1 h at 50 °C. The cotton fabric was treated in the next step by the above described dispersion. The soaked fabric was squeezed with an 85% spin effect and air dried. The as-prepared cotton fabric was added, in the next step, to the mixture of 2-propanol (100 g) and TEOS (20 g), mixed well, and left for 10 min at 50 °C. Then, a solution of ammonia (7 g) in water (20 g) was added to the TEOS solution, which was re-mixed again and left for 1 h at 50 °C. The immersed cotton textile was taken out of the reaction mixture, rinsed with water three times and dried at room temperature. This was followed by applying a 10% PDMSU-FAS solution, performing the impregnating procedure with full soaking, squeezing with an 85% spin effect, drying at 100 °C and curing at 150 °C for 5 min.

## Claims

1. A process for the preparation of self-cleaning wash-resistant, air permeable, superhydrophobie, oleophobic and self-cleaning cotton textiles, which includes the following steps:
- modifying the cotton fabrics in advance with a deposition of pre-prepared first type of spherical SiO₂ particles, wherein the modification is carried out using aqueous/alcoholic dispersions of spherical SiO₂ particles 200 - 1000 nm in size;
- applying a second type of spherical SiO₂ particles by an *in-situ* sol-gel method, wherein the second type of spherical SiO₂ particles is grown *in-situ* on the surface of textile fibres from a colloidal nucleus dispersion during which the *in-situ* formation of spherical SiO₂ particles of the second step with a size between 50 and 200 nm occurs and wherein the whole surface of the textile is covered with the same bi-hierarchical roughness through the formation of a thin porous coating, which enables the chemical bonding of the first type of spherical SiO₂ particles, deposited in the first step, to the surface of cotton fabrics;
- the rough cotton surface is further consolidated by application of a sol-gel coating prepared from hydrophobic and oleophobic silanes.

2. The process according to claim 1 **characterized in that** at least 95% of the first type of spherical SiO₂ particles in the dispersion are of the same size, the concentration of dispersed spherical SiO₂ particles is 10% by weight, and the ratio of the weight of the dispersed spherical SiO₂ particles and the mass of the textile is 1:15.

3. The process according to claim 1 and 2 **characterized in that** the chemical bonding of the spherical SiO₂ particles deposited in the first step with the surface of cotton fabrics is enabled by the reactivity of the free-OH groups on the spherical SiO₂ particles and the textiles.

4. The process according to claims 1 to 3 **characterized in that** for the preparation of spherical SiO₂ particles in the first and second step organic-modified silanes are used, such as tetraethoxy ortosilane, methyltriethoxysilane, vinyltriethoxysilane or aminopropyltriethoxysilane, preferably tetraethoxy ortosilane.

5. The process according to claims 1 to 4 **characterized in that** the weight ratio of the pre--prepared spherical SiO₂ particles in the first step and the spherical SiO₂ particles prepared *in-situ* during the second step is between 1:2 and 1:3.

6. The process according to claims 1 to 5 **characterized in that** for the hardening of a roughened surface hydrophobic and oleophobic silanes are used which are selected from perfluoroalkyl-trialkoxysilanes, perfluoroalkyl-alkyldialkoxysilanes, perfluoroalkyl-dialkylalkoxysilanes, perfluoroalkyl-trihalosilanes, perfluoroalkyl-alkyldihalosilanes, perfluoroalkyl-dialkylhalosilanes, and (trialkoxysilyl)alkyl terminated polydimethylsiloxanes.

7. The process according to claims 1 to 6 **characterized in that** the thickness of the thin layer of the hydrophobic and oleophobic silanes may not exceed 150 nm.

8. The process according to claims 1 to 7 **characterized in that** the coating of individual layers on the surface of cotton fabrics is applied by exhaustion method, by dipping, or by sputter deposition.

## Patentansprüche

1. Verfahren zur Herstellung waschbeständiger, luftdurchlässiger, superhydrophober, oleophober und selbstreinigender Baumwolltextilien, umfassend die folgenden Schritte:
- Modifizierung der Baumwollgewebe im Voraus mit einer Abscheidung von voraufbereiteten sphärischen SiO₂-Partikel erster Art, wobei die Modifizierung unter Verwendung von wässrigen/alkoholischen Dispersionen kugelförmiger SiO₂-Partikel mit einer Größe von 200-1000 nm erfolgt;
- Aufbringen einer zweiten Art von kugelförmigen SiO₂-Partikeln durch ein *in-situ* Sol-Gel-Verfahren, wobei der zweite Typ von kugelförmigen SiO₂-Partikeln *in-situ* auf der Oberfläche der Textilfasern aus einer kolloidalen Keimdispersion wächst , bei der die *in-situ* Bildung von kugelförmigen SiO₂-Partikeln des zweiten Schritts mit einer Größe zwischen 50 und 200 nm erfolgt und wobei die gesamte Gewebeoberfläche durch die Bildung einer dünnen, porösen Beschichtung mit der gleichen bihierarchischen Oberflächenrauigkeit erfolgt, die die chemische Bindung des ersten Typs von kugelförmigen SiO₂-Partikeln, die im ersten Schritt abgeschieden wurden, auf die Oberfläche von Baumwollgeweben ermöglicht;
- die rauhe Baumwolloberfläche wird durch Aufbringen einer aus hydrophoben und oleophoben Silanen hergestellten Sol-Gel-Beschichtung weiter verfestigt.

2. Verfahren nach Anspruch 1, **dadurch gekennzeichnet, dass** mindestens 95% der ersten Art der kugelförmigen SiO₂-Partikel in der Dispersion gleich groß sind, die Konzentration an dispergierten kugelförmigen SiO₂-Partikeln 10 Gew.-% beträgt, und das Verhältnis des Gewichts der dispergierten kugelförmigen SiO₂-Partikeln zu der Masse des Textils 1 : 15 beträgt.

3. Verfahren zur Herstellung nach Anspruch 1 und 2, **dadurch gekennzeichnet, dass** die chemische Bindung der im ersten Schritt abgeschiedenen kugelförmigen SiO₂-Partikeln mit der Oberfläche von Baumwollgeweben durch die Reaktivität der freien OH-Gruppen an den kugelförmigen SiO₂-Partikeln und der Textilien ermöglicht wird.

4. Verfahren nach den Ansprüchen 1 bis 3, **dadurch gekennzeichnet, dass** zur Herstellung von kugelförmigen SiO₂-Partikeln organisch-modifizierte Silane, wie Tetraethoxysilan, Methyltriethoxysilan, Vinyltriethoxysilan oder Aminopropyltriethoxysilan, vorzugsweise Tetraethoxysilan eingesetzt werden.

5. Verfahren zur Herstellung nach den Ansprüchen 1 bis 4, **dadurch gekennzeichnet, dass** das Gewichtsverhältnis der zuvor im ersten Schritt hergestellten kugelförmigen SiO₂-Partikeln und der im *in-situ* Verfahren hergestellten kugelförmigen SiO₂-Partikeln zwischen 1:2 und 1:3 beträgt.

6. Verfahren zur Herstellung nach den Ansprüchen 1 bis 5, **dadurch gekennzeichnet, dass** zur Härtung von hydrophoben und oleophoben Oberflächen Silane eingesetzt werden, die aus Perfluoralkyldialkylalkoxysilanen, Perfluoralkyltrialkoxysilanen, Perfluoralkylalkyldihalogensilanen, Perfluoralkyldialkylhalogensilanen und (Trialkoxysilyl) alkylterminierten Polydimethylsiloxanen ausgewählt werden.

7. Verfahren nach den Ansprüchen 1 bis 6, **dadurch gekennzeichnet, dass** die Dicke, der dünnen Schicht der hydrophoben und oleophoben Silane, 150 nm nicht überschreiten darf.

8. Verfahren nach den Ansprüchen 1 bis 7, **dadurch gekennzeichnet, dass** die Auftragung der einzelnen Schichten auf die Oberfläche von Baumwollgeweben durch Ausziehverfahren, Tauchen oder durch Sputterabscheidung erfolgt.

## Revendications

1. Procédé pour la préparation de textiles en coton autonettoyants, résistants au lavage, perméables à l'air, superhydrophobes, oléophobes et autonettoyants, qui comprend les étapes suivantes :
- modification à l'avance des tissus en coton par déposition de particules sphériques de SiO₂ pré-préparées, la modification étant réalisée à l'aide de dispersions aqueuses/alcooliques de particules sphériques de SiO₂ de taille de 200 à 1000 nm ;
- application d'un second type de particules sphériques de SiO₂ par un procédé sol-gel *in situ,* le second type de particules sphériques de SiO₂ étant mis à croître *in situ* sur la surface de fibres textiles à partir d'une dispersion de noyaux colloïdaux, au cours de laquelle se produit la formation *in situ* de particules sphériques de SiO₂ de la seconde étape avec une taille comprise entre 50 et 200 nm et la surface entière du textile étant recouverte de la même rugosité bihiérarchique par la formation d'un revêtement poreux mince, qui permet la liaison chimique du premier type de particules sphériques de SiO₂, déposées au cours de la première étape, sur la surface de tissus en coton ;
- la surface de coton brut est en outre consolidée par application d'un revêtement sol-gel préparé à partir de silanes hydrophobes et oléophobes.

2. Procédé selon la revendication 1, **caractérisé en ce qu'**au moins 95% des particules sphériques de SiO₂ dans la dispersion ont la même taille, la concentration des particules sphériques de SiO₂ dispersées est de 10 % en poids, et le rapport entre le poids des particules sphériques de SiO₂ et la masse du textile est de 1 : 15.

3. Procédé selon les revendications 1 et 2, **caractérisé en ce que** la liaison chimique des particules sphériques de SiO₂ déposées au cours la première étape avec la surface de tissus en coton est permise par la réactivité des groupes OH libres sur les particules sphériques de SiO₂ et les textiles.

4. Procédé selon les revendications 1 à 3, **caractérisé en ce que** pour la préparation de particules sphériques de SiO₂ aux première et seconde étapes, des silanes modifiés organiques sont utilisés, tel que le tétraéthoxy ortosilane, le méthyltriéthoxysilane, le vinyltriéthoxysilane ou l'aminopropyltriéthoxysilane, de préférence le tétraéthoxy ortosilane.

5. Procédé selon les revendications 1 à 4, **caractérisé en ce que** le rapport pondéral entre les particules sphériques de SiO₂ préalablement préparées à la première étape et les particules sphériques de SiO₂ préparées *in-situ* au cours de la deuxième étape se situe entre 1 : 2 et 1 : 3.

6. Procédé selon les revendications 1 à 5, **caractérisé en ce que** pour le durcissement d'une surface rugueuse, des silanes hydrophobes et oléophobes sont utilisés qui sont choisis parmi les perfluoroalkyl-trialcoxysilanes, les perfluoroalkyl-alkyldialcoxysilanes, les perfluoroalkyl-dialkylalkoxysilanes, les perfluoroalkyl-trihalogénosilanes, les perfluoroalkyl-alkyldihalosilanes, les perfluoroalkyl-dialkylhalosilanes, et les polydiméthylsiloxanes à terminaison (trialcoxysilyle) alkyle.

7. Procédé selon les revendications 1 à 6, **caractérisé en ce que** l'épaisseur de la couche mince de silanes hydrophobes et oléophobes ne doit pas dépasser 150 nm.

8. Procédé selon les revendications 1 à 7, **caractérisé en ce que** le revêtement de couches individuelles sur la surface de tissus en coton est appliqué par procédé d'épuisement, par trempage, ou par dépôt par pulvérisation cathodique.
